

## UNITED STATES PATENT OFFICE

RALPH H. PRICE, OF CHICAGO, ILLINOIS, ASSIGNOR, BY MESNE ASSIGNMENTS, TO GLUE RESEARCH CORPORATION, OF NEW YORK, N. Y., A CORPORATION OF NEW YORK

## GLUE SOLUTION AND PROCESS OF MANUFACTURING SAME

No Drawing.

Application filed December 7, 1925. Serial No. 73,919.

My invention relates to a new composition of matter and it has special reference to an improved glue solution and the process of producing the same.

5 More particularly my invention relates to a new solution comprising glue, which solution possesses a slight tendency only to jell but yet contains a high concentration of glue. By means of my invention I am able to produce a glue solution having a relatively high 10 glue content and which possesses a considerably lower jelling point for a given concentration of glue than an ordinary water solution containing substantially the same percentage of the same grade of glue.

My present solution, as exemplified by the specific illustrative solutions of my invention hereinafter described, has only a slight tendency to form a jelly at 70° F. and it does not undergo bacterial decomposition under ordinary 20 conditions of storage and use. When the solution of my present invention, as exemplified by the specific illustrative solutions hereinafter to be described, is applied to a 25 surface, the solution dries very quickly because of the relatively high content of volatile organic solvent. By reason of the greater fluidity of my glue solution under ordinary conditions of use, it appears to have 30 more penetrating and spreading power than a water solution having substantially the same glue concentration. These advantages particularly obtain with my new glue solution when applied to wood, fabrics, paper or 35 other absorbent materials.

The ordinary animal glues dissolved in water form viscous solutions which vary in fluidity with the concentration and other factors for the particular grade of glue used. 40 Such glue solutions tend to form a jelly upon standing at room temperature unless extremely dilute and, unless some preservative is added, putrefaction due to bacterial decomposition soon sets in which alters considerably the strength and other properties 45 of the glue. In my present glue solution bacterial decomposition is substantially precluded and, therefore, my improved glue solution retains many of its initial properties.

50 Other objects of my invention will be here-

inafter revealed and for a better understanding of my invention reference may now be had to the following description and the appended claim which define my invention.

My invention is applicable to the production of glue solutions adapted to many industrial uses. The following procedure may be used to produce a solution especially adapted to wood finishing. Inasmuch as different grades of glue varying in viscosity, 55 jell strength, acidity, etc. may be required for other uses of my improved solution, it is, of course, to be understood that the proportions which I herein specify are not essential but may be varied in accordance with 60 the requirements for which the glue solution is to be adapted.

As a specific illustrative solution of my invention, I may utilize a clear glue which gives no precipitate with ferric ammonium 70 sulphate by the method of testing described below, which glue is of the commercial grade known as "Glue Association grade 4-4" and which has a jelly test of substantially 85 grams or lower and a viscosity test of substantially 35 millipoises or lower, both of these tests being conducted in accordance with the official methods of the National Association of Glue Manufacturers as published in "Industrial and Engineering Chemistry", vol. 16, No. 3, p. 310. This glue is 80 soaked in cold water in the proportion of substantially five parts of glue to four parts of water by weight. After the glue has swelled thoroughly, which will require only 85 two or three hours if a ground glue is used, this mixture is heated in a water jacketed kettle for a sufficient period to produce a smooth solution. I mix in a separate vessel one part of glycerine and two parts of denatured ethyl alcohol by weight.

For the proportions mentioned above, in still another vessel I dilute five parts of denatured ethyl alcohol with two parts of water by weight. Having prepared these three 95 solutions I now take three parts of the alcohol-glycerine mixture and to it I add slowly eight parts of the hot aqueous glue solution, while constantly stirring the mixture. This mixture comprising the various ingredients 100

is then stirred with sufficient vigor to produce a smooth solution and while still stirring I slowly add eight parts of the diluted alcohol. The solution is then strained or filtered 5 carefully to remove therefrom any foreign matter. (It should now be and should remain quite fluid at room temperature and should be substantially free from lumps or flocculated material.) It is to be understood 10 that the order of addition of the above substances may be changed and other modifications may be made in the above technique without departing from the spirit and scope of this invention.

15 Glue is not a simple chemical compound but a very complex mixture of protein compounds and other substances of a nitrogenous nature, which mixture varies widely in the commercial product. In view of this fact it 20 may be necessary to slightly vary the above proportions with different glues, even though they show the same jell and viscosity tests. A satisfactory solution may be obtained with any glue of the above description by substituting for part of the alcohol an equal amount of water. All proportions given above are by weight.

While a glue showing no precipitate with ferric ammonium sulphate, such as is specified 25 in the illustrative solution given above, produces a thoroughly satisfactory solution it is to be understood that other glues not responding to this test can be used, although slight modifications in the formula may be necessary. 30 Solutions prepared from such glues may show under certain conditions a slight precipitate but will still be wholly satisfactory for certain purposes.

The method of performing the ferric ammonium sulphate precipitation test on glue 40 is as follows: Twenty grams of the glue is soaked in 80-100 grams of cold distilled water for three hours. It is then heated at about 60° C. on a water bath until a smooth solution 45 is obtained, after which it is diluted to 500 cubic centimeters with distilled water. A water solution of ferric ammonium sulphate is made up to contain 10 grams of this salt per 100 grams of solution. The ferric ammonium sulphate mentioned is the crystalline salt containing 24 molecules of water of crystallization. When to 100 cubic centimeters of the above dilute aqueous glue solution is 50 added 20 cubic centimeters of the ferric ammonium sulphate solution no precipitate, or 55 at least only a faint turbidity, should develop, even on stirring, after allowing the mixtures to stand at about 70° F. for 12 hours.

Throughout this specification and the 60 claims it is to be understood that the word "glue" as used herein includes any commercial adhesive of animal origin, such as the alkaline casein glue composition as well as glue from fish, hides, bones, etc. It is well 65 known that commercial glues made from fish,

hides, bones, etc. are substantially neutral in reaction although because of the crude methods commonly used for the adjusting of these glues to neutrality, the commercial products are frequently either very faintly acid or alkaline.

A solution similar in properties to the solution mentioned in the above example may be prepared using casein. Inasmuch as casein lacks uniformity in quality and cannot usually be purchased on such definite jell and viscosity specifications, as is the case with "animal glues," the proportions given in the following example are to be understood as being only approximate.

As an example using casein, I take 50 parts of water and in it dissolve 3 parts of soda ash. To this is added slowly with stirring, 28 parts of dry casein. The mixture is allowed to stand until the casein has swelled somewhat and is then heated in a water jacketed vessel until a smooth solution is obtained. In a separate vessel, a mixture of equal parts of denatured ethyl alcohol and neutral 75% Turkey red oil is heated to approximately 120° F. and 16 parts of this warm mixture is added slowly with constant stirring to the alkaline casein glue mixture. More alcohol, first warmed to about 120° F., is now added.

With certain caseins which I have used, I have found it possible to add 50 parts of alcohol at this point without precipitation taking place in the finished solution. It will be understood, however, that because of the great variation in the quality of commercial casein available it will be necessary to determine, for the casein to be used, just how much alcohol can be added without causing an undesirable precipitate in the finished product.

105 All proportions in this example also are by weight.

The alcohol which I have described above as being "denatured ethyl alcohol" is designated in the trade as "Number 5 completely denatured alcohol" and contains per 100 parts by volume of ethyl alcohol, 2 parts by volume of methyl alcohol, one fourth part by volume of pyridine bases, one half part by volume of benzine and usually about 4-6 110 parts by volume of water. However, ethyl alcohol denatured in certain other ways may be used if desired.

115 Sulphonated or water soluble vegetable or mineral oils, glucose or similar glue softening substances, or mixtures of these substances or mixtures of these substances with glycerine, with Turkey red oil or with both glycerine and Turkey red oil may be used in proper proportions in place of the glycerine or Turkey red oil specified in the above illustrative examples. Such ingredients provide a highly satisfactory solution for most purposes, although for certain uses it is possible to prepare a useful but less satisfactory

80

75

85

90

95

100

105

110

115

120

125

130

glue solution without them. As a specific illustration of such a glue solution, applicant may utilize a clear glue of the commercial grade known as Glue Association grade 4-4 such as was used in the example hereinbefore cited in the specification. This glue is soaked in cold water in the proportion of substantially five parts of glue to four parts of water by weight. After the glue has swelled thoroughly it is heated in a water jacketed kettle until a smooth solution is obtained. In a separate vessel seven and one-half parts of denatured ethyl alcohol may be mixed with three and one-half parts of water. This dilute alcohol is then added very slowly to the above concentrated aqueous glue solution while the whole is rapidly and vigorously agitated. In this coating composition, the glue softening agent is absent.

Instead of denatured ethyl alcohol I may use, among others, the following water soluble organic solvents; methyl alcohol; iso propyl alcohol; other water soluble higher alcohols; acetone, and water soluble esters. I may also use water soluble mixtures of the above-mentioned solvents. When I use substantially water insoluble solvents, such as methyl acetate; ethyl acetate; other substantially water insoluble esters; turpentine; furfural or mixtures of these, I add thereto such of the above described water soluble organic solvents as will produce a resultant water soluble solvent. The relative proportions of these substances may be varied with the grade of glue chosen and the purpose for which this solution is to be used.

As stated above, one use to which my improved glue solution may be applied advantageously is in finishing wood. Under such circumstances, the glue solution may be applied with a pneumatic spray brush or by other means thereby producing an undercoat or liquid filler. When the glue solution dries, it is almost entirely insoluble in such solvents as are found in varnishes, paints, and in nitro-cellulose lacquers. This insolubility minimizes the tendency for the lacquer or varnish to be drawn into the grain of the wood or into the texture of any similar absorptive material to which my glue solution may be applied. In this fashion, a considerable saving is effected in the number of required coats of finishing materials, such as lacquer or varnish. Since my glue solution dries very rapidly, it is usually possible to apply any subsequent coat or coats of finishing material within two or three hours or less after applying the last glue undercoat. This is highly advantageous in this art when this time interval between coats is compared with the time interval which usually has been required heretofore with the former fillers and undercoats.

Another advantage possessed by my glue

solution is that it does not appreciably raise the grain of wood as is done by the usual water solutions, as heretofore employed. Therefore sanding is eliminated in most cases although the surface may be sanded easily if desired.

Still another advantage possessed by my glue solution in the wood finishing art is that it effectively seals in the stain which may have been applied previously to the wood undergoing treatment. As a result, this prevents the solvents in the lacquer or varnish from dissolving the stain which process produces an unsightly appearance. At present, shellac is commonly used as a sealing coat to prevent this so-called "bleeding" of the stain, but shellac is not always effective because of the partial solubility of the shellac in the usual lacquers or varnishes. Consequently, the stain may still bleed through the shellac coat to some extent. When my glue solution is used as a sealing coat for stained work, it is preferable not to sandpaper the coat because it is highly desirable to preserve the glue coat as a continuous unbroken film.

Another use to which my present glue solution may be put is to provide a good paste wood filler or plastic composition which is capable of hardening. When used for this purpose I mix with my glue solution finely pulverized silica or other inert filler material, and pigments or stain, if desired.

Another use to which my glue solution may be put is to adapt it as a binding substance for clay, pigments or other materials in the manufacture of wallpaper or coated papers where an adhesive material is desired which will not require being kept warm continuously during use.

Because of the lesser tendency of my present glue solution to jell at room temperature, and its greater penetrating power for a given concentration of the glue, my solution is a desirable adhesive for wood joining, for plywood and veneer manufacture, and in the manufacture of laminated or plastic molded products. Furthermore, the glue in my solution may be hardened and made relatively waterproof by treatment in the usual way with such hardening agents as formaldehyde, paraformaldehyde, chromium salts and the like and by the application of heat. Such a hardening treatment is of advantage in some of the above-mentioned applications for my glue solution. When hardened and waterproofed in this fashion my solution may be used as a finish coat for various materials such as wood, paper and the like.

While I have herein described my present invention and the process of manufacturing the same, as well as methods for using my new glue solution, it is to be understood that various modifications may be made therein.

without departing from the spirit and scope  
of the appended claim.

I claim:

5 A freely fluid sprayable albuminoid coating composition comprising a non-jelling  
stable solution of substantially 29 parts of  
commercial glue substantially free from  
foreign acid reacting substances in a solvent  
comprising substantially  $33\frac{1}{3}$  parts by  
10 weight of ethyl alcohol and substantially 35  
parts of water, and an amount equivalent to  
substantially one-tenth of the weight of the  
glue of a glue plasticizing agent selected from  
15 the group consisting of glycerol and Turkey  
red oil.

In witness whereof I have hereunto sub-  
scribed my name.

RALPH H. PRICE.

20

25

30

35

40

45

50

55

60

65